

Dec. 24. 1935.

W. A. WISSLER

2,025,368

MOUNTING ALLOY DIES

Filed Sept. 23, 1931



Fig. 1



Fig. 2



Fig. 3

INVENTOR:  
William A. Wissler,  
BY  
Patten, Pierce & Schaffler,  
ATTORNEYS.

## UNITED STATES PATENT OFFICE

2,025,368

## MOUNTING ALLOY DIES

William A. Wissler, Jackson Heights, N. Y., assignor to Haynes Stellite Company, a corporation of Indiana

Application September 23, 1931, Serial No. 564,711

3 Claims. (Cl. 22—204)

The invention relates to a method of mounting dies, and has particular reference to a mounting for extremely hard alloy dies of the type used in wire drawing.

5 In the use of dies of extremely hard, and more or less brittle alloys, it is customary to reinforce the die by mounting it in a body of supporting metal. The supporting or mounting metal not only serves to reinforce the die, but being of softer metal than the die, it may be more easily formed and shaped into any desired size to suit the apparatus in which the die is to be used. Heretofore the usual manner of mounting has consisted in pressing the die into a ring, shrinking on an outside casing, or casting a metal such as bronze around the die in the shape desired. Mountings of this sort are not entirely satisfactory, since they do not give sufficient support to prevent the die from cracking under normal usage, and especially under any severe strain.

It is an object of my invention to provide a more efficient manner for mounting alloy dies, which will permit their use without danger of cracking under the strains of the ordinary drawing operation, and will also permit the use of certain alloys as dies which heretofore were entirely unsatisfactory for that purpose when mounted in the usual manner, due to their tendency to crack.

30 In accordance with my invention the mounting is formed about the die in such a manner that the mounting metal and the alloy of the die actually unite with each other at their contacting surfaces to form a union resembling a weld. When the mounting consists of bronze or other of the metals commonly used in brazing operations, the joint between the mounting and the die might more correctly be termed a brazed union. But since other metals than those used for brazing 35 may be equally suitable as a mounting, I prefer throughout the specification and claims to refer to my process as a particular form of welding operation, although it will be understood that the union between the two metals is not necessarily 40 a true autogenous weld.

45 Many of the metals or alloys heretofore used for mounting will, under the conditions of my method, properly weld with the die alloy. Metals having a high elastic limit at high temperatures, and a coefficient of expansion higher than the 50 alloy of the die, are especially suitable. Bronze, a copper-nickel alloy such as "Monel metal", or steel have all been found to be satisfactory. In applying the mounting metal the die may be 55 located and held in a crucible or other container

in a position which will permit the formation about the die of a mounting having the shape desired. The mounting metal, in the form of solid particles, is then introduced into the refractory container or crucible, along with a suitable flux, and heat is applied to completely melt the metal into place about the die. A mounting metal or alloy is used which has a much lower fusion point than the alloy of the die, so that it may be completely reduced to a molten condition 5 without fusing the die, or in any way altering the size or shape of the die hole. The flux used should be one capable of cleaning the surface of the die, and the temperature should preferably be carried to a point somewhat higher than the 10 melting point of the mounting metal. On cooling the mounting metal shrinks to a much greater extent than the die, which causes a tension to be set up in the mounting. The elasticity of this metal however is sufficient to hold this tension 15 until the unit is entirely cold. Thus a die assembly is formed in which the mounting is not only welded to the surface of the die, but also acts to support and reinforce it under tension.

20 The method has been found to be especially 25 suitable for mounting tungsten alloy dies of the type whose extreme hardness may be attributed to the presence of certain amounts of tungsten carbide. These dies, which will be referred to as tungsten carbide dies, are admirably suited in 30 hardness to resist the frictional wear of wire drawing, but they do not have sufficient strength to resist cracking when mounted in the manner heretofore used. I prefer as a mounting metal 35 for such dies an alloy of substantially the composition, copper 65%, nickel 31%, iron 1%, and manganese 3%. The die is placed in a crucible in the manner previously described, and the mounting metal and a borax flux are distributed about the die. The crucible is then placed in a 40 furnace and heated to a temperature of approximately 1200° C. This temperature is sufficient 45 thoroughly to fuse the surrounding alloy, whereby the fluid metal fills the unconfined space about the die. The flux acts to clean the surface of the die, and the metal of the mounting welds with this surface, although there appears to be no actual fusion of the die alloy. As previously explained, the mounting cools under tension. This 50 tension, along with the welded contact of the two alloys, so reinforces the die as to permit the use 55 of tungsten carbide dies in drawing operations where heretofore they were of little or no value, due to their tendency to crack.

A typical form of the invention is shown in the drawing, in which

Figures 1 and 2 represent two stages in the process of mounting an alloy die, and

Figure 3 is a mounted die.

Referring to Figure 1, a graphite crucible 10 may be used as the refractory container. Within the crucible 10 may be placed a removable graphite block 11 having a centrally located point or projection to aid in centering the die. A die-blank 12, provided with a centering-hole or depression, is placed on the block 11, flux and pieces of metal are placed in the crucible, and the whole then placed in a furnace to fuse the said metal.

Upon removal from the furnace, the die is found to be surrounded with metal 13, as shown in Figure 2. The contents of the crucible 10 are then allowed to cool, and when cool are removed from the crucible. The mounting metal 13 is then turned down to the desired shape and size, and the die 12 is drilled.

In Figure 3, the drilled die 12 is shown surrounded by the turned mounting metal 13.

Although especially applicable to tungsten carbide dies, the invention may also be useful in mounting many other types of dies which have extreme hardness, but which must be reinforced by means of a mounting. Various modifications in the particular procedure described may also be made without departing from the spirit of my invention, especially with reference to the manner of placing and fusing the mounting metal to form the shape desired. For example the mounting metal or alloy may be melted about the die, and welded thereto by means of an ordinary welding flame or torch while supported in most any type of a suitable container. The invention should not be limited other than as defined in the appended claims.

I claim:

1. A method of mounting alloy dies which com-

prises placing the die in a refractory container, disposing about said die solid particles of a mounting composition consisting chiefly of copper and nickel and having a higher coefficient of expansion and a higher elastic limit at high temperatures than the alloy of the die, adding thereto a flux adapted to clean the surface of the die, and heating the container to a temperature such that the mounting composition is completely fused and welding occurs at the contacting surfaces of the die and the mounting, whereby the die is securely bonded to the mounting and re-enforced by the effect of the high elastic tension which is set up in the mounting, and breaking of the die when in use is minimized.

2. A method of mounting tungsten carbide dies which comprises placing the die in a refractory container, disposing about said die a mounting composition comprising copper, nickel, iron and manganese, said composition having a higher elastic limit at high temperatures, a higher coefficient of expansion, and a lower melting point than said die material, adding thereto a flux adapted to clean the surface of the die, and heating the container to a temperature such that the mounting composition is completely fused and welding occurs at the contacting surfaces of the die and the mounting, whereby during cooling of the mounting the elasticity thereof is sufficient to withstand the tension created by the unequal contraction of the die and the die mounting, and fracturing of the die when in use is minimized.

3. A method of mounting tungsten carbide dies which comprises placing the die in a refractory container, disposing about said die a mounting metal having substantially the composition, copper 65%, nickel 31%, iron 1%, and manganese 3%, adding thereto a borax flux, and heating the container to a temperature of about 1200° C., whereby the mounting metal welds with the surface of the die.

WILLIAM A. WISSLER.